

## UNITED STATES PATENT OFFICE.

STANLEY M. UDALE, OF DETROIT, MICHIGAN, ASSIGNEE TO EARL HOLLEY, OF DETROIT, MICHIGAN.

## IRON MOLD.

No Drawing.

Application filed November 22, 1925. Serial No. 71,018.

This invention relates to an improved cast iron permanent mold. The object of this invention is to devise a mold which will have the minimum degree of expansion and the maximum degree of life, consistent with a high degree of fluidity when molten. When steel contains 36% of nickel its expansion has been found to be not much more than 25% of the normal expansion up to a temperature of about 500° F.

Steel, however, is not a very satisfactory metal to use because it is not sufficiently fluid to form cast molds, which is the object of this invention, and if these molds have to be machined out of the solid the expense is such that the mold cost per casting becomes appreciable and there is then no saving over casting in sand.

In order to raise the fluidity of iron a considerable percentage of carbon is added which lowers the melting point. In order that the iron should be soft when cast it is desirable to throw the carbon out of solution with the silicon. Iron containing a large amount of carbon in solution is liable to distortion during the operation of repeatedly casting iron in it. The reason for this is that the increase of temperature necessary when pouring molten iron into an iron mold causes the mold to expand because graphite has less than 50% of the specific gravity of iron and therefore when it comes out of solu-

tion the volume of the entire mass increases and surface cracks develop, and ultimately the mold disintegrates.

I have found that gray iron containing 2.6% silicon, 3.0% carbon, a total of manganese, phosphorus and sulphur equal to 1%, and 93.4% iron is a satisfactory material for the molds. As nickel has a tendency to precipitate carbon, the silicon can be lowered to 2.0%. In order to secure a steel alloy of 36.0% nickel in this cast iron, the cast iron must contain, therefore, a percentage of nickel of 34.5%, of iron 61.4%, of carbon 2.0%, of silicon 1.3%, and the balance (0.8%) will consist of manganese, sulphur and phosphorus. The carbon is chiefly in the free state, the objection to combined carbon being as stated.

What I claim is:—

1. A cast mold containing 34.5% nickel, 61.4% iron, 2.0% carbon (mostly free), 1.3% silicon, and 0.8% of manganese, sulphur, and phosphorus.
2. A cast mold containing between 30% and 40% nickel.
3. A cast mold containing from 34% to 38% nickel and the balance chiefly iron with a little carbon, silicon, manganese, phosphorus, and sulphur.

In testimony whereof I affix my signature.

STANLEY M. UDALE.